

## UNITED STATES PATENT OFFICE

2,219,320

HEAT TREATING PROCESS FOR WHITE  
CAST IRON

Collet Jones, Lafayette, Ind.

No Drawing. Application July 22, 1939,  
Serial No. 285,955

4 Claims. (Cl. 148—21.7)

This invention relates to a heat-treating process for white cast iron, by which such white cast iron may be given improved properties; and to the product of such process. This application is a continuation in part of my co-pending application Serial No. 76,294, filed April 24, 1936.

White cast iron has been used as such in a limited way, but its properties are so poor, except in respect to its extreme hardness and wear resistance, that it has comparatively few engineering applications. It has low strength, is brittle, has no ductility, may not be worked, and is machinable only with great difficulty. Its primary use, other than when it is remelted and converted into a product such as steel, is as a basis for malleable iron, which is the cheapest form into which white cast iron may be changed. To produce malleable iron, the white cast iron is cast into the desired pieces, and such castings are heated to a temperature well above the critical point of the material, are held at that temperature for a period of days, and are then very slowly cooled. The process is long, and requires expensive furnace and heating equipment, so that it is itself quite expensive.

In the malleabilization process, the carbon which appears in the original white cast iron in the form of cementite is transformed into graphite which appears as nodules distributed substantially throughout the finished product. Thus, malleable iron has a matrix of substantially carbon-free iron with graphite particles distributed therein.

In the present process, it is my object to give the white cast iron different properties than are given to it by the malleabilization process and which in many respects are better qualities than those in malleable iron. It is a further object of my invention to secure these improved properties by a relatively simple and short process.

Microscopic examination shows the product to have a matrix of iron and cementite with the cementite thereof largely in spheroidized form, and that the additional carbon which is present is in the form of substantially disconnected particles or masses of massive cementite.

The product has substantially improved properties. Its tensile strength is above 75,000 and usually above 80,000 pounds per square inch or more. The product is readily machinable, it may be forged at a temperature of about 1400° to 1460° F. and may be welded with either an electric arc weld or an acetylene weld. It has a high resistance to abrasion, and takes a high polish. It may be given subsequent heat treatments such

as those applied to steel, to cause changes in the properties of the carbon containing matrix similar to those which occur in steel.

In general, the process is performed upon white iron castings by heating them in a furnace to a temperature substantially above the  $Ac_1-3$  point of the material, holding them at that temperature for a period of time, the temperature and the holding time being sufficient to cause some of the cementite to go into solution in the austenite and to secure at least partial diffusion and equalization in the austenite, so that there is formed a substantially homogeneous matrix of substantially saturated austenite. The temperature and holding time, however, is insufficient to cause any substantial formation of graphite either during such holding or during subsequent steps in the process. The castings are then furnace cooled to a temperature between 700° and 800° F., at which temperature they should be held a sufficient time to equalize the temperature throughout the body of the white cast iron; and are then quenched, preferably in water.

The heating may be done at as rapid a rate as convenient, but with the usual precautions against warpage. The temperature to which they are heated should be above the  $Ac_1-3$  point of the white cast iron, in order to secure the formation of austenite to dissolve cementite, and should be considerably above such point. On the other hand, the temperature should not be so high that graphite will form or that too great a tendency toward graphitization will occur. I have found that the temperature should be between about 1600° and 1700° F.

The time during which the metal is held at this high temperature after the furnace has been brought to the high temperature should be in accordance with the usual practice in the heat treatment of steel, to permit the austenite to dissolve more cementite and to permit diffusion and equalization of the cementite which is dissolved in the austenite. That is, the time during which the metal is held at the desired high temperature, from the time the furnace reaches such temperature, should be for approximately one hour for each inch of metal, calculated in accordance with usual heat-treating practice.

At the conclusion of the holding time, the metal is cooled at a relatively slow rate, but fast enough to avoid graphitization. Preferably, it should be furnace cooled, as by permitting the pieces to remain in the furnace and to cool with the furnace, or by removing the pieces from the high-temperature furnace and immediately

charging them in a furnace which is held at the temperature to which they are to be cooled. Expressed in cooling rates, I have found that the cooling should not be below about 25° F. per hour and may be faster, up to about 1000° F. per hour, these cooling rates being average cooling rates and not necessarily uniform throughout the cooling operation.

The cooling is carried to a temperature of about 700° to 800° F., most desirably 720° F., is held there for any period necessary to equalize the temperature of the piece at that point, and may be held a longer period at that temperature. If the cooling is in the range of about 250° to 400° F. per hour, and the castings are small, the holding period at the 700°-800° F. temperature may be omitted.

At the conclusion of the cooling and any low-temperature holding time, the castings are rapidly quenched, preferably in a liquid quenching medium; and I have found that a water quench gives best results.

A study of this process, and of the product thereof, indicates that metallurgically the process acts as follows: When the white cast iron reaches its  $Ac_1$ - $3$  temperature, its pearlitic portions form austenite in which is dissolved the cementite from such portions. As the iron is heated more and held at 1600°-1700° F., the austenite dissolves cementite from the excess which is present. In the untreated white cast iron, this excess cementite occurs largely in the form of thin layers or stringers, which form a network through the original material, and also in the form of larger and relatively thick masses. At the high temperature the austenite becomes substantially saturated, a large part of the stringers are dissolved, especially at their thinner portions, and diffusion and equalization of the dissolved cementite throughout the austenite occurs. This eliminates the coarse dendritic structure, and breaks up the net work of relatively weak and brittle cementite, to give a more continuous matrix of austenite with the undissolved and disconnected cementite masses distributed through it.

The heat treatment is not so severe nor so long continued that graphite is formed, although I believe a tendency toward graphite formation is unavoidably set up during the heating necessary to get a desirable amount of the cementite in solution and diffused.

During slow cooling above the  $Ar_1$ - $3$  point the excess cementite separates not in its original stringer form but instead in a more spheroidized form. At the  $Ar_1$ - $3$  point the austenite is changed to pearlite, which during the continued cooling is itself at least partially spheroidized. There is thus formed a matrix of pearlite and spheroidized cementite, which is substantially continuous although it has embedded in it the undissolved masses of cementite which are now substantially disconnected.

As has been stated, during the treatment of the white iron castings at the high temperature, I believe there is a tendency set up for graphite to be formed. If the cooling is carried to room temperature at the slow rate, the graphite actually separates out, and its presence in any substantial amount materially weakens the resulting product. Quenching from the desired temperature of approximately 720° F., however, substantially prevents this formation of graphite.

The slow cooling to the quenching temperature produces in the matrix properties of toughness and ductility, and makes the product readily

machinable. Because of the substantial absence of graphite particles and the discontinuity of the massive cementite, the material may be forged.

The following are examples of my process:

*Example 1.*—Test bars of  $\frac{5}{8}$  inch diameter were used which had an analysis as follows:

|             | Per cent |
|-------------|----------|
| Carbon      | 2.40     |
| Silicon     | 1.00     |
| Manganese   | 0.35     |
| Phosphorous | 0.155    |
| Sulphur     | 0.075    |

This analysis is believed to be typical of commercial white cast iron, and the test bars upon examination showed structures typical of high grade clean white cast iron.

Several of these test bars were placed in a cold furnace and heated in about 1½ hours to a temperature of 1675° F. and held at that temperature for about 30 to 45 minutes. The current was then shut off and the furnace allowed to cool to 720°. The cooling took about 3½ hours so that the average cooling rate was about 270° per hour. When a temperature of 720° had been reached the test bars were removed from the furnace and immediately quenched in water at room temperature. The resulting bars had an average tensile strength of about 80,000 pounds per square inch, they were machined and found to be readily machinable, they were subjected to relatively severe forging, and were found capable of being satisfactorily formed in this way. Untreated bars were similarly forged and were found wholly incapable of withstanding such treatment. Samples of the treated bars were welded in a forge fire, others were welded by acetylene, and others by the use of an electric arc, with satisfactory results. The metal was found capable of taking a high polish upon being machined and ground, and was readily drilled with a plain carbon steel drill of No. 60 size.

*Example 2.*—Test bars similar to those of Example 1 were placed in a furnace and heated for about 1½ hours at which time their color indicated that they had attained a temperature of about 1600°-1700° F. and were held at that temperature for thirty minutes. The metal was then permitted to cool in the furnace as rapidly as it would, and when the metal changed color from red heat to black heat in cooling, the operator started stroking one of the pieces of metal in the furnace with a file. When the metal showed a bright mark when stroked with the file the bars were removed from the furnace and quenched in water. Subsequent tests disclosed that when the metal showed a bright mark when stroked with the file the temperature was about 720° F. The bars treated in this run were tested in a manner similar to those of Example 1 and found to have substantially the same properties.

*Example 3.*—Several variously sized commercial white iron castings were carefully loaded in a container in such a way that the weight of the several pieces would not tend to deform them, and the container was placed in a furnace and heated to about 1700° F. The pieces were held at this temperature for a time calculated at the rate of one hour for each inch of metal of the thicker portions of the castings. The furnace was then permitted to cool to a temperature of approximately 720° F., during which time the charge was withdrawn two or three times for short examination periods.

The castings were held at 720° F. for about the same time as the holding time at the high temperature, and were then quenched in water.

The resulting treated castings were compared 5 in various respects with the known properties of identical pieces which had been malleabilized and were found satisfactory for commercial use. The process had been performed under non-production conditions within about eleven hours, while 10 the malleabilizing process applied to the comparative pieces normally took a period of five days.

I claim as my invention:

1. A process to quick anneal white iron castings with the aid of a water quench in the short 15 cycle of time of 5½ hours or less, said process involving heating the white iron casting for about 1½ hours until it attains a temperature of approximately 1675 degrees F. thereby to get a more homogeneous condition by eliminating the 20 coarse dendritic structure, then maintaining the heat at this temperature until the transformation takes place, then cooling the casting in the furnace at a rate of 250 degrees F. to 400 degrees F. per hour until it reaches a temperature of approximately 25 720° F., and then immediately quenching the casting in water.

2. A process for the treatment of white cast iron, which comprises heating the white cast iron to a temperature of approximately 1600° F. to 30 1700° F., holding it at that temperature to secure substantial saturation of the austenite, furnace cooling it at a rate of from 250° F. to 400° F.

per hour to between 800° F. and 700° F., and then subjecting it to a rapid quench from that temperature.

3. A heat-treating process for white cast iron, comprising heating the white cast iron to a temperature substantially above its  $Ac_{1-3}$  temperature and holding it at such temperature to cause austenite to be formed and to dissolve a substantial part of the original stringer formation of massive cementite and to secure a more homogeneous condition of the matrix but substantially avoiding graphite formation both during such holding and in subsequent process operations, subjecting the cast iron to cooling conditions in a temperature not below about 700° F. until it reaches a uniform temperature of approximately 700° to 800° F., and quenching the cast iron from the temperature to which it is cooled.

4. A heat-treating process for white cast iron, comprising heating a white-iron casting to a 20 temperature of about 1600° to 1700° F., holding it at that temperature a time sufficient to cause a considerable portion of the stringer formation of cementite to be dissolved while substantially avoiding graphitization, cooling the cast iron at 25 a rate of between about 250° and 1000° F. per hour to a temperature of about 700° to 800° F., holding it at such temperature any time necessary to secure a uniform temperature in it, and quenching it from that temperature.

5

15

20

25

30

COLLET JONES.